

## UNITED STATES PATENT OFFICE

2,133,435

## TEXTILE THREAD AND FABRIC

William Alexander Dickie and Robert Wighton  
Moncrieff, Spondon, near Derby, England, as-  
signors to Celanese Corporation of America, a  
corporation of Delaware

No Drawing. Original applications May 17, 1932,  
Serial Nos. 611,922 and 611,924. Divided and  
this application October 20, 1936, Serial No.  
106,614. In Great Britain June 4, 1931

10 Claims. (Cl. 117—21)

This invention relates to the manufacture of  
textile fabrics and textile threads suitable for  
incorporation therein. The application is a di-  
visional application of our applications S. Nos.  
5 611,922 and 611,924 both filed 17th May, 1932,  
which have issued as Patent Nos. 2,089,947 and  
2,089,948, respectively.

Textile materials exhibiting crêpe effects have  
long been obtained by employing in their con-  
10 struction highly twisted yarns of natural silk  
in the gummed state, the crêpe effects appearing  
more particularly when the fabric is subjected to  
scouring in an aqueous bath. The fabrics ob-  
tained by this process have long been highly val-  
ued on account of their pleasing appearance and  
15 handle. The production of crêpe fabrics in an  
analogous manner by the use of highly twisted  
yarns of cellulose acetate filaments has however  
been accompanied by very considerable difficul-  
20 ties. In many cases it is found that little or no  
crêpe effect is obtained unless a very consider-  
able degree of twist is imparted to the crêpe  
threads. Further, when this degree of twist is  
25 sufficient to lead to the production of crêpe ef-  
fects comparable with those obtainable by means  
of natural silk, it is found that the strength of  
the resulting fabrics is frequently so low as to  
render them commercially valueless.

We have now found that in utilizing highly  
30 twisted cellulose acetate yarns in the manufac-  
ture of crêpe fabrics a great improvement, par-  
ticularly as regards the strength of the finished  
fabrics, may be effected by subjecting the yarn  
35 to the action of water vapour or by wetting the  
yarn with water or other aqueous liquid before  
at least part of the crêpe twist is applied thereto.  
For example a cellulose acetate yarn of about  
100 denier and containing about 25 filaments  
40 may be twisted to 25 to 30 turns per inch or more  
and then subjected to the action of steam at  
about 60—105° C., i. e. under a pressure below  
or slightly above that of the atmosphere, or then  
45 wetted thoroughly with water. The so treated  
yarn is thereafter twisted to 60—70 turns per inch  
and utilized as the weft of a fabric, pairs of picks  
of right-hand twist alternating with pairs of  
picks of left-hand twist. The fabric may then  
50 be scoured and finished, whereupon a fabric ex-  
hibiting excellent crêpe effects and of very good  
properties as regards strength may be obtained.  
If the treatment with steam or water is omitted  
55 the resulting fabrics may exhibit a serious re-  
duction in strength in the direction of the highly  
twisted yarns.

55 In the manufacture of the crêpe threads in

accordance with our invention, the requisite high  
degree of twist is thus applied in at least two  
stages with intermediate treatment of the yarn  
with water vapour or with water or other aqueous  
liquid. If desired the twisting may be accom-  
plished in three or more stages, the yarn being  
wetted or treated with water vapour between  
any or all of the stages. Further, if desired, the  
yarn may be subjected, in addition, to water va-  
pour treatment before twisting or after the total  
amount of twist has been applied.

The degree of twist employed in the crêpe  
threads may vary within wide limits and ac-  
cording to the nature of the yarn and of the  
filaments contained therein. Thus, for instance,  
a total twist of from 55 to 65 or 70 turns per  
inch may be employed, though higher twist may  
be employed if desired, for example a twist of  
80—85 or more turns per inch. Yarn composed  
of fine filaments is advantageous in that it ad-  
mits of the use of a very high degree of twist.

The total twist may be applied either in equal  
or in unequal stages. Thus, where twisting is  
to be effected in two stages, half the twist may  
be applied in each, or a small or large proportion  
in the first stage and in the second stage the cor-  
responding proportion required to give the de-  
sired total twist. Thus, for instance, where the  
total twist is to be 65 turns per inch, the yarn  
may first be twisted to 10 turns per inch, then  
steamed or wetted, and thereupon an additional  
55 turns per inch applied to give the necessary  
total twist. Again, if desired 40 turns per inch  
may first be applied and 25 turns per inch in  
the second stage. In an analogous manner when  
three or more stages are employed the twist may  
be divided between the various stages in any  
desired manner. As indicated previously, how-  
ever, in the case of yarn of about 100 denier and  
containing about 25 filaments very good results  
40 may be obtained by applying about 25 turns per  
inch in the first stage.

In practice, it has been found particularly ad-  
vantageous to apply in the first place a degree of  
twist of the order of that necessary to cause a  
close packing of the filaments of the yarn and  
then to treat the latter with water vapour or wa-  
ter and thereafter to impart the degree of twist  
necessary to give rise to crêpe effects of the de-  
sired character. In the case of 100 denier 26 fila-  
ment yarn the desired close packing is secured  
by the application of about 25 turns per inch.  
It will be appreciated that the exact degree of  
twist necessary to give the desired close packing  
of the filaments is dependent in any particular  
50 55

case on the total denier of the yarn and the number of the filaments of which it is composed. Thus for yarns of a given total denier the twist required to effect close packing is greater the 5 smaller the number of filaments. Again, for yarns containing a given number of filaments the desirable first stage twist varies inversely as the diameter of the filaments or the square root of the filament denier. In general for yarns of 10 between 70 and 170 denier and containing from 25 to 70 filaments the degree of twist applied before the wetting operation will be between about 10 and 30 turns per inch.

The twisting of the yarns may be effected in 15 any convenient manner. It has been found advantageous however, particularly when applying the second or subsequent stage of twist, to utilize twisting devices of the type in which the yarn is twisted as it is drawn off from a rotating pack- 20 age and to prevent the applied twist running back to the bobbin. This result may very conveniently be attained by means of the device described in U. S. Patent No. 1,784,581.

The crêpe effects obtained appear to be de- 25 pendent chiefly upon the degree of twist im- parted after the steam or water treatment and are to some extent independent of the degree of twist applied before the steam or water treat- 30 ment particularly if the said degree of twist is not much below that required to effect close pack- 35 ing of the filaments. It has in fact been found that the character or extent of the crêpe effects finally obtained in the fabrics may be controlled to some extent by varying the proportion of 40 twist applied after a steaming or wetting treat- ment. The amount of twist imparted in the final stage or stages following packing of the filaments into a firm thread will thus depend to a certain extent on the denier of the yarns and on the 45 type of crêpe effect to be produced. In general a good figure is obtained on the fabrics by the use of a total twist of 60-65 to upwards of 85 turns per inch.

In the treatment of the yarns in accordance 45 with the present invention, the steam may be employed under any desired pressure and at any desired temperature, for example at pressures below or slightly above that of the atmosphere, and at temperatures corresponding to the boil- 50 ing point of water at those pressures. The steam may be saturated or wet. Very good results may be obtained for instance by using steam at pres- 55 sures up to 5 lbs. per square inch below or above atmospheric pressure, though higher pressures, for example 10-20 lbs. per square inch or more, may be used if desired. Water may be applied to the yarns at a temperature of 80° C. up to or even above the boiling point.

The yarns may be steamed or treated with 60 hot water in the course of one of the twisting operations utilized to apply the requisite twist to the yarn. Conveniently the yarn may be passed through a suitable chamber which may for instance take the form of a tube supplied 65 with steam of the desired temperature. If de- 70 sired the steam may be applied to the yarn at the point at which the twist is actually applied. For this purpose, in the case of using a twisting machine of the type in which twist is applied as the yarn is drawn off from a bobbin or like 75 package, the thread guide immediately above the bobbin from which the yarn is drawn off may be mounted at the point of entry of the yarn into the tube or like chamber in which the steam is applied, or the thread guide may actually be

within the said tube or like chamber. Preferably the steam is applied only in the minimum quantity necessary to secure the desired effect on the yarn in order that escape of steam and the consequent likelihood of troubles arising from the 5 rusting of machinery and the like may be avoided as far as possible.

If desired hygroscopic or deliquescent sub- 10 stances or wetting agents i. e. agents facilitating the wetting of solids by water, may be applied to or incorporated in the yarns prior to a twisting operation or a steaming or wetting treatment. As examples of such wetting agents may be mentioned soaps of organic or inorganic bases with higher fatty acids, for example alkali metal, 15 ammonium or ethanolamine soaps, sulphonated oils, sulphonic acids of alkyl naphthalenes for example butyl naphthalene sulphonic acid, and sulphonic acids or sulphuric esters of higher aliphatic alcohols or of mineral oils, tar oils and 20 the like. Mention may also be made of wetting agents of a basic character, for example the higher poly-amines of the aliphatic series and basic derivatives of the higher fatty acids, for instance oleyl derivatives of aliphatic diamines or 25 other higher fatty acid derivatives of this character.

Such hygroscopic or deliquescent substances or wetting agents may be applied to the yarns, or if desired may be incorporated in spinning 30 solutions from which the yarns are prepared. For example, cellulose acetate solutions containing hygroscopic substances, for instance sodium or potassium acetate or calcium or magnesium chloride or nitrate may be spun into filaments 35 and the latter formed into yarns and treated in accordance with the invention.

Such wetting agents may be applied in con- 40 junction with the hot water used for a wetting treatment.

After the operation of steaming or wetting with hot water the yarn may be allowed to stand for a time. In order to obtain a thread capable of giving rise to crêpe effects, further twist is applied to the yarn directly or after subjecting the 45 yarn to a drying operation in order to remove a part or the whole of any moisture content.

However, after the twisting operation effected while the thread is under the influence of steam or hot water, i. e. at a stage when the twist in the thread is insufficient to impart crêping 50 power to the thread, the thread is per se useful and moreover the process of producing such a thread is novel, i. e. the process which consists in applying to the thread while under the in- 55 fluence of steam or hot water a twist insufficient to impart crêping power thereto. The purpose of the present divisional application is to claim the production of these threads having a twist lower than a crêping twist by this novel process. 60

We have further found that hot water may be applied in the form of a fine spray. Thus for instance during the twisting operation, a very fine spray of heated water may be applied to the yarn. Such spray of water may be applied 65 in restricted quantities so as to avoid as far as possible any rusting of the machinery. The spray may for instance be applied in a closed chamber, for example a chamber of tubular form through which the yarn is passed. The 70 apparatus previously referred to as suitable for use in applying steam may be employed if desired.

If desired lubricants may be applied to the 75 yarns which are to receive the twist, especially

while the yarns have no twist or at any rate only a low degree of twist. Such lubricant, for example, olive oil or castor oil or oleic acid, assists the filaments to slide easily over each other so that they may more readily take up their proper position in the yarn, particularly during the early stages of twisting, prior and up to the point at which close packing is reached. Such lubricant may be permitted to remain in the yarns throughout the twisting, when it may be removed after incorporation of the yarns in fabrics.

The invention is of particular value in connection with the production of fabrics with the aid of yarns consisting of cellulose acetate filaments.

5 Yarns comprising filaments of other organic derivatives of cellulose may be employed in an analogous manner. As examples of such cellulose derivatives may be mentioned cellulose formate, propionate or butyrate or other cellulose esters 10 of organic acids, or methyl, ethyl or benzyl cellulose or other cellulose ethers. If desired yarns consisting of or comprising filaments of other materials may be employed, for example filaments of silk, cotton, or of artificial silk of the 15 regenerated cellulose type. The yarns may also be composed of filaments of two or more different kinds whether in respect of material or denier or both. Thus there may be used threads containing both filaments of cellulose esters or ethers 20 and filaments of natural silk or regenerated cellulose artificial silk, or threads containing cellulose ester or ether filaments of two or more different deniers, or threads containing filaments of one cellulose derivative e. g. an ester in admixture with filaments of another cellulose derivative e. g. an ester of different ester content or an ether. Further the yarns may consist, wholly or in part, of "staple fibre", i. e. relatively 25 short lengths of filaments.

30 The threads may be incorporated in the fabrics in any suitable manner, for example the weft alone may be wholly or partially composed of such threads or the warp may also contain them. They may be disposed in the fabrics in any convenient manner, for example pairs of 35 threads of left-hand twist may alternate with pairs of threads of right-hand twist.

What we claim and desire to secure by Letters Patent is:—

50 1. Process for the manufacture of textile threads, which consists in twisting the thread to a degree lower than a creping twist and applying a hot aqueous fluid to the thread during the actual insertion of said twist, the total twist applied to the thread being insufficient to impart creping power thereto.

55 2. Process for the manufacture of textile threads, which consists in twisting the thread to a degree lower than a creping twist and applying steam to the thread during the actual insertion of said twist, the total twist applied to the thread being insufficient to impart creping power thereto.

60

the thread being insufficient to impart creping power thereto.

3. Process for the manufacture of textile threads, which consists in applying twist to a thread to a degree lower than a creping twist 5 and steaming the thread during the actual insertion of said twist, the total twist applied to the thread being insufficient to impart creping power thereto.

4. Process for the manufacture of textile 10 threads, which consists in applying twist to a thread to a degree lower than a creping twist whilst the thread is under the influence of wet steam, the total twist applied being insufficient to impart creping power to the thread. 15

5. Process for the manufacture of textile threads, which consists in applying twist to a thread of cellulose acetate filaments to a degree lower than a creping twist and steaming the thread at the point at which said twist is actually 20 applied, the total twist applied being insufficient to impart creping power to the thread.

6. Process for the manufacture of textile threads, which consists in twisting a thread composed of artificial cellulosic filaments to a degree 25 lower than a creping twist and applying a hot aqueous fluid to the thread during the actual insertion of said twist, the total twist applied to the thread being insufficient to impart creping power thereto. 30

7. Process for the manufacture of textile threads, which consists in twisting a thread composed of artificial cellulosic filaments to a degree lower than a creping twist and applying steam to the thread during the actual insertion of said 35 twist, the total twist applied to the thread being insufficient to impart creping power thereto.

8. Process for the manufacture of textile threads, which consists in twisting a thread composed of artificial cellulosic filaments to a degree 40 lower than a creping twist and applying wet steam to the thread during the actual insertion of said twist, the total twist applied to the thread being insufficient to impart creping power thereto.

9. Process for the manufacture of textile threads, which consists in twisting a thread composed of cellulose acetate filaments to a degree 45 lower than a creping twist and applying a hot aqueous fluid to the thread during the actual insertion of said twist, the total twist applied to the thread being insufficient to impart creping power thereto. 50

10. Process for the manufacture of textile threads, which consists in twisting a thread composed of cellulose acetate filaments to a degree 55 lower than a creping twist and applying wet steam to the thread during the actual insertion of said twist, the total twist applied to the thread being insufficient to impart creping power thereto.

WILLIAM ALEXANDER DICKIE.

ROBERT WIGHTON MONCRIEFF.

60